

## UNITED STATES PATENT OFFICE.

KARL W. J. H. JACOBS, OF HAMBURG, GERMANY.

## LOW-TEMPERATURE DISTILLATION OF CARBONIZABLE MATERIAL.

No Drawing. Application filed August 24, 1921, Serial No. 494,785, and in Germany July 28, 1919.

(GRANTED UNDER THE PROVISIONS OF THE ACT OF MARCH 3, 1921, 41 STAT. L., 1313.)

The present application relates to a new or improved process for the improvement of inferior brown coals and peat, and deals in particular with the treatment of materials, 5 such as very woody lignite of fibrous or fragmentary structure, which can only be briquetted with difficulty, if at all.

The process consists in subjecting the material to a restricted dry distillation in which 10 it is not completely coked but only attains an intermediate condition between coal and coke. The completely distilled coke obtained from such material is somewhat inferior, partly on account of its low inflammability and the 15 consequent restricted usefulness, and partly by reason of its usually low cohesion.

According to the present invention a readily ignitable and valuable heating material with a heating value of about 6000 calories 20 or more, can be obtained from a crude coal of barely 2000 calories, by interrupting the coking process prior to its final stage. The process is carried out as follows (the temperatures given are centigrade).

25 The more or less pre-dried crude coal is first freed from water and the bulk of the carbon dioxide at a progressively increasing temperature. As soon as the temperature exceeds about 250 deg., the first tarry distillates 30 can be observed, and at about 270 deg., an exothermic reaction begins, by means of which the distillation is continued. By this means and the further application of heat, additional quantities of low-temperature tar pass 35 over into the receiver. The heating is then increased until the temperature is between 290 and 350, during which interval the low-temperature tar in all the coals examined is driven over. A few kinds of coal require 40 temperatures of up to 350 deg. At this point the heating is interrupted after the low-temperature tar has passed over. The resulting material is a valuable long-flame fuel,

which is more particularly useful for furnaces. A maximum yield of valuable low- 45 temperature tar is obtained as a by-product. In view of the poor heat conductivity of the material to be treated, it may be advisable in the interests of uniform heating—especially in retorts of large diameter—to supplement 50 the external application of heat by an internal heating with superheated steam.

However, in order that the yield of fuel may not suffer in the interests of the yield 55 of gas, not more than 10% of steam (based on the weight of the material under treatment) should be used. This small quantity of steam is sufficient to ensure that the charge will be warmed through in a uniform manner and to accelerate the removal of the distillation gases from the retorts so as to prevent overheating. In addition, the yield of ammonia and acetic acid, together—although to a smaller extent—with that of methyl alcohol, is increased. 60

## I claim:—

The process of treating moist, solid carbonizable material containing appreciable quantities of oxygen and capable of releasing by chemical decomposition substantial 70 quantities of tarry material when heated to temperatures between 250° C. and 350° C. and substantial quantities of tarry material of a different character when heated to temperatures above 350° C. which comprises, heating said material in a distilling retort to dry the same, progressively raising the temperature thereof up to about 350° C. and then cooling the residue while removing volatilized material from the retort while said residue 75 still contains a major portion of tar forming material capable of releasing tar at temperatures above 350° C. 80

In testimony whereof I affix my signature.

KARL W. J. H. JACOBS.